

## UNITED STATES PATENT OFFICE.

JOHANN EV. KOLLINGER, OF MUNICH, GERMANY.

## PAINT AND PROCESS OF MAKING SAME.

SPECIFICATION forming part of Letters Patent No. 738,456, dated September 8, 1903.

Application filed February 7, 1903. Serial No. 142,401. (No specimens.)

*To all whom it may concern:*

Be it known that I, JOHANN EV. KOLLINGER, merchant, a citizen of Bavaria, Germany, residing at Munich, Bavaria, Germany, (whose 5 post - office address is Lindwurmstrasse, 24/III,) have invented certain new and useful Improvements in Paint and Process of Making Same; and I do hereby declare the following to be a full, clear, and exact description 10 of the invention, such as will enable others skilled in the art to which it appertains to make and use the same.

My invention relates to an improvement in paints and the process of making the same.

15 The object of my invention is to produce a paint which while weatherproof and capable of resisting the effects of the sun's rays will flow readily under the brush when being applied, will not show the marks of the brush, 20 and will dry with a beautiful dead gloss, distinguishing this paint from all others.

With this general object in view my invention consists in a paint whose vehicle or binding medium is formed from a composition of 25 mineral, animal, and vegetable oils mixed with resin, as more particularly pointed out hereinafter.

My invention consists, further, in the process of making said paint.

30 In carrying out my invention I preferably proceed as follows: I melt eight to fourteen parts, by weight, of tallow with fourteen to twenty-four parts of a vegetable oil, such as linseed-oil, and to this I add a composition 35 formed by mixing two hundred to two hundred and thirty parts, by weight, of a mineral oil, such as petroleum, thirty to fifty parts of melted tallow, fifty to seventy parts of a vegetable oil, such as linseed-oil, and fifty to 40 seventy parts of a resin, intimately mixing this composition by stirring. To this vehicle or binding medium the desired pigment may be added, preferably in a powdered form, the whole being then ground or rubbed together 45 until thoroughly commingled. The product is then ready for use and will be found to be easily applied and absolutely weatherproof when dried. These advantages are still further heightened by the modification of my 50 invention substantially as follows: To the binding medium prepared as above I add the desired pigment and then a composition of a

vegetable oil, saponified resin, and turpentine, for instance. To two hundred and thirty to three hundred and twenty parts of the 55 binding medium prepared as above is added twenty to fifty parts of a vegetable oil, such as linseed-oil, fifteen to forty parts of saponified resin, and five-tenths to four parts of turpentine, the whole being thoroughly ground 60 or rubbed to unite the ingredients. Obviously the before-mentioned composition, consisting of a vegetable oil, saponified resin, and turpentine, may be added also preferably to the binding medium prepared as above described—*i. e.*, before adding the pigment to said binding medium. 65

Paint prepared in accordance with my invention has many advantages over the ordinary paint in that it spreads or flows well 70 under the brush, thus being readily laid on and leaving a smooth surface which does not show the brush-marks. Furthermore, the coat, which is absolutely weatherproof and will not blister even under the hottest rays of the 75 sun, will become in some months as hard as a lake color.

It is to be understood that the binding medium or vehicle disclosed by me may be prepared without the addition of the pigment 80 and kept in stock ready to be united with any desired color previous to applying.

Having thus fully described my invention, what I claim as new, and desire to secure by Letters Patent, is— 85

1. The process which consists in melting tallow and vegetable oil together, then adding a mineral oil and a resin, and intimately mixing the composition. 90
2. The process which consists in melting tallow and vegetable oil together, then adding a mineral oil, melted tallow, a vegetable oil and a resin, and intimately mixing the composition. 95
3. The process which consists in melting together tallow and a vegetable oil in the proportions of eight to fourteen parts of tallow and fourteen to twenty-four parts of vegetable oil, then adding a mineral oil, melted tallow, a vegetable oil and a resin, and intimately mixing the composition. 100
4. The process which consists in melting together tallow and a vegetable oil in the proportions of eight to fourteen parts of tallow

with fourteen to twenty-four parts of vegetable oil, then adding two hundred to two hundred and thirty parts of a mineral oil, thirty to fifty parts of melted tallow, fifty to seventy parts of a vegetable oil, and fifty to seventy parts of resin, and intimately mixing the composition.

5. The process which consists in melting together tallow, and a vegetable oil, then adding a mineral oil, melted tallow, a vegetable oil and a resin, intimately mixing the composition, and thereupon adding the desired coloring-matter.

6. The process which consists in melting together eight to fourteen parts of tallow with fifteen to twenty-four parts of a vegetable oil, then adding a composition formed by uniting two hundred to two hundred and thirty parts of a mineral oil, thirty to fifty parts of melted tallow, fifty to seventy parts of a vegetable oil and fifty to seventy parts of a resin, then intimately mixing the composition, next adding the desired coloring-matter, then rubbing or grinding the composition.

25 7. The process which consists in melting together tallow and a vegetable oil, then adding a mineral oil, melted tallow, a vegetable oil and a resin, intimately mixing the composition, adding the desired coloring-matter, then uniting this composition with vegetable

oil, saponified resin and turpentine and thoroughly grinding or rubbing the mixture.

8. The process which consists in melting together tallow and a vegetable oil, then adding a mineral oil, melted tallow, a vegetable oil and a resin, intimately mixing the composition, then mixing two hundred and thirty to three hundred and twenty parts of the so-prepared mixture with twenty to fifty parts of a vegetable oil, fifteen to forty parts of saponified resin and five-tenths to four parts of turpentine, and thoroughly grinding or rubbing the mixture.

9. The composition of matter containing tallow, vegetable oil, mineral oil, resin and turpentine.

10. The composition of matter consisting of tallow, vegetable oil, mineral oil, and saponified resin.

11. The composition of matter consisting of tallow, vegetable oil, mineral oil, resin, and saponified resin.

12. The composition of matter, containing tallow, a vegetable oil, a mineral oil, a resin, a pigment, a saponified resin and turpentine.

In testimony whereof I affix my signature in presence of two witnesses.

JOHANN EV. KOLLINGER.

Witnesses:

WALTER E. BOWMAN,  
CLARA I. PARKER.